

(No Model.)

2 Sheets—Sheet 1.

J. T. ROWLEY.  
METHOD OF PRODUCING HOLLOW INGOTS.

No. 603,206.

Patented Apr. 26, 1898.

Fig. 1



Fig. 2



WITNESSES:

William J. Brown  
G. A. Williams

John T. Rowley, INVENTOR  
BY J. H. Brown  
His  
ATTORNEY.

(No Model.)

2 Sheets—Sheet 2.

J. T. ROWLEY.  
METHOD OF PRODUCING HOLLOW INGOTS.

No. 603,206.

Patented Apr. 26, 1898.

Fig. 3



Fig. 4



Fig. 5



WITNESSES:

William J. Brown.  
C. A. Williams

John Thomas Rowley, INVENTOR  
BY J. T. Rowley, his  
ATTORNEY.

# UNITED STATES PATENT OFFICE.

JOHN THOMAS ROWLEY, OF BEAVER FALLS, PENNSYLVANIA.

## METHOD OF PRODUCING HOLLOW INGOTS.

SPECIFICATION forming part of Letters Patent No. 603,206, dated April 26, 1898.

Application filed May 27, 1897. Serial No. 638,355. (No model.)

*To all whom it may concern:*

Be it known that I, JOHN THOMAS ROWLEY, a citizen of the United States, residing at Beaver Falls, in the county of Beaver and State of Pennsylvania, have invented certain new and useful Improvements in Methods of Producing Hollow Ingots; and I do hereby declare the following to be a full, clear, and exact description of the invention, such as will enable others skilled in the art to which it pertains to make and use the same, reference being had to the accompanying drawings, which form a part of this specification.

My invention relates to a certain new method of manufacturing hollow ingots, which I shall describe with reference to the accompanying drawings, in which is shown a form of device or apparatus preferably adapted to the application of my invention or discovery. In the drawings, Figure 1 indicates a front elevation of said machine. Fig. 2 is a plan view of the same. Fig. 3 is an end view of the same. Fig. 4 is a vertical transverse section of the same. Fig. 5 shows a longitudinal section and end view of an ingot produced by my method.

The device herein illustrated is in many respects similar to the machine patented by me by Letters Patent No. 566,701, dated August 25, 1896. I will therefore not describe the same in detail, but only in so far as the same varies from that shown in said Letters Patent.

Referring to said drawings, A is a horizontal cylindrical roll mounted in suitable housings B B and adapted to be adjusted with reference to the concave die-plate C by the bars or rods D D, the said roll being arranged with reference to said concave back or plate, parallel therewith longitudinally and preferably slightly eccentric to the contour thereof, so that the opening-pass between the top of said roll and the inner face of said concave plate is somewhat greater than the exit-pass between the said two surfaces, so that the reduction of the ingot increases progressively from the entrance to the exit-pass.

In the practice of my method I take a heated blank or ingot and place the same in the pass between the roll and the concave die-plate, the sides of said solid ingot being parallel with the faces of the roll and the die-

plate. The rotation of the roll causes said ingot to move progressively down the pass between the roll and the die-plate, the same being, as shown in the drawings, of gradual decreasing width. The ingot in its progressive movement through the pass is constantly rotated on its own axis, the draft or friction on the surfaces of the same being sufficient to gradually reduce the same in cross-section. By this operation, which may be repeated if necessary, the ingot is seemingly stretched peripherally while it is being reduced in diameter and increased in length, thus gradually forming a hollow ingot.

My method consists, broadly, in first heating a solid bar or ingot, preferably octagonal or round in cross-section, then subjecting it to the friction or pressure of two or more surfaces parallel with the axis of the ingot being operated upon, the bar or ingot being during the operation free to rotate on its own axis, the billet or bar being free to elongate, and this operation continued and the distance between the surfaces decreased, if necessary, until, as before stated, the solid bar is formed into a hollow ingot of less cross-section and greater length than the solid ingot. In the practice of my method all of said surfaces may be rotary, as when a series of rolls are used, or one of said surfaces may be fixed and stationary, as in the form of device illustrated in the drawings. In either case the draft on the surface of the ingot must be sufficient to produce a constantly-decreasing diameter and an elongation of the bar or ingot.

I have reduced my invention to practice.

Having described my invention, what I claim, and desire to secure by Letters Patent, is—

1. The herein-described improvement in method for producing hollow ingots from solid bars or billets, which consists of heating the solid ingot, bar, or billet and subjecting the same to the friction or pressure of a plurality of surfaces parallel with the axis of the billet, the billet or bar being free to rotate on its axis and to elongate during the operation, substantially as described.

2. The herein-described improvement in method for producing hollow ingots from solid bars or billets, which consists of heating the bar or billet and subjecting the same to the

friction or pressure of a plurality of surfaces, the said surfaces being parallel with the axis of the bar or billet and adapted to progressively increase the reduction of the ingot, the 5 ingot or bar being free to rotate on its axis and to elongate during the operation, substantially as described.

3. The herein-described improvement in method for producing hollow ingots from solid 10 bars or billets, which consists in first heating the solid ingot, subjecting the same to the

pressure of a roll and a vertical concave die-plate, the billet or bar being free to rotate on its axis and to elongate during the operation, substantially as described. <sup>15</sup>

In testimony that I claim the foregoing I hereunto affix my signature this 25th day of May, A. D. 1897.

JOHN THOMAS ROWLEY. [L. S.]

In presence of—  
JAS. J. MCABEE,  
C. A. WILLIAMS.